

# United States Patent Office

2,764,550

Patented Sept. 25, 1956

1

2,764,550

## GEAR-OIL LUBRICANTS

Joseph B. Stucker, Des Plaines, Norman D. Williams, Chicago, and George Wolfram, Union, Ill., assignors to The Pure Oil Company, Chicago, Ill., a corporation of Ohio.

No Drawing. Application February 24, 1951,  
Serial No. 212,694

4 Claims. (Cl. 252—46.6)

The present invention relates to lubricating compositions having extreme pressure characteristics and more particularly to lubricants for gears such as hypoid gears, transmissions and differentials.

In United States Patents 2,211,306 and 2,483,571, there are disclosed and claimed processes for making extreme pressure additives for use in lubricating oil compositions. These extreme pressure additives are made by sulfurizing a fatty body or fatty oil and then phosphorizing the sulfurized product so produced. Extreme pressure additives made in accordance with these patents have been successfully used for many years and have proven highly satisfactory. These extreme pressure additives, when made from ordinary fatty oils, as for example lard oil, have one disadvantage and that is their lack of solubility and compatibility with solvent refined hydrocarbon oils and with Pennsylvania bright stocks. This lack of compatibility with these lubricating oil fractions leads to instability of the finished lubricating composition during storage.

Since the majority of lubricating oil fractions presently available and being used for compounding are the solvent refined variety and since Pennsylvania bright stocks are highly desirable constituents the problem was presented to ascertain why the sulfurized-phosphorized fatty oils were insoluble therein. The lack of solubility of extreme pressure additives was found to be due to the presence of high molecular weight polymers in the finished product. It was found that if the starting material used in the preparation of the extreme pressure additive was an ester of a dihydroxy alcohol and a mono-ethenoid acid of the general formula  $C_nH_{2n-2}O_2$  containing from 10 to 24 carbon atoms in the molecule instead of the triglyceride type of material such as lard oil, this difficulty was eliminated. Examples of suitable starting esters are mono- or di-esters of propylene glycol or butylene glycol. The use of these esters as starting materials for the sulfurization-phosphorization reaction not only solved the problem of compatibility with these lubricating oil stocks but also improved the pour characteristics of the finished product. This development is the subject matter of two copending applications bearing Serial Number 653,438, filed March 9, 1946, now Patent No. 2,542,161, and Serial Number 740,723, filed April 10, 1947, now Patent No. 2,541,789, by one of the co-inventors herein.

The special extreme pressure additives prepared from these special esters are quite expensive and for this reason it is highly desirable that a way be found to increase the solubility and compatibility of extreme pressure additives in solvent refined and Pennsylvania bright lubricating oil stocks by less expensive means.

The present invention is based upon discovery that a lubricating oil composition containing the solvent refined lubricating oil base stocks or the Pennsylvania bright stocks may be made compatible with the less expensive sulfurized-phosphorized fatty oil extreme pressure additives by incorporating as a part of the composition a product from the solvent extraction or refining of lubricating oils. This product, as will be seen, not only enhances the compatibility characteristics of the finished gear oil, but also replaces a part of the more expensive lubricating oil portion of the composition. Other advantages of the

2

invention will be seen as the description thereof proceeds.

Accordingly the main object of this invention is to provide a means for solubilizing sulfurized-phosphorized fatty body extreme pressure agents in the presence of solvent refined lubricating oil bright stocks and bright stock from Pennsylvania oils.

A second object of this invention is to provide a base oil which exhibits satisfactory solubility and compatibility for extreme pressure additives, especially sulfurized-phosphorized fatty body extreme pressure agents.

A third object of this invention is to provide a new universal gear oil containing sulfurized-phosphorized fatty body extreme pressure agent, blends of neutrals with solvent refined bright stock and/or a Pennsylvania bright stock in a compatible, homogeneous composition.

The fourth object of this invention is to provide a gear oil lubricating composition which meets the requirements of United States Army Specification MIL-L-2105.

A further object of this invention is to provide a new superior blended gear oil composition containing solvent extract from lubricating oil stocks.

Other objects and advantages of this invention will become apparent as the description thereof proceeds.

The extraction products above referred to which are to be incorporated as part of gear oil compositions in accordance with this invention, are obtained from the solvent extraction of lubricating oils. After the fixed gases, gasoline, naphtha, kerosene and light lubricating fractions have been removed by fractionation from a crude oil, the reduced crude so produced is deasphalting. The deasphalted oil is next extracted with a solvent to produce highly refined aviation lubricating oils and resultant solvent extract used in accordance with this invention. For example, a Van Zandt crude oil with an API gravity of 33.1 was topped to remove such light fractions as gasoline, naphtha, kerosene and a light lubricating distillate. The vacuum residue was a reduced crude having a viscosity of 1251 SUS at 210° F., 2.2% sulfur and API gravity of 12.6. This reduced crude was deasphalting by treatment with propane yielding a deasphalted oil having a viscosity at 210° F. of 174 SUS and API gravity of 21.7. The deasphalted oil was treated with phenol to produce a raffinate from which an aviation lubricating oil may be produced. The extract from this phenol treatment is ready for use in blending or additive production in accordance with this invention without further processing.

Other solvents than phenol may be used to obtain the extraction product used in accordance with this invention, for example, furfural or the Duo-Sol solution comprising liquid propane, phenol and cresol may be used. When using phenol it is possible to vary the characteristics of the extraction product considerably by adjustment of the amount of water present. For example, a low V. I. cut may be obtained by using a water solution of phenol during the extraction and a high V. I. cut may be obtained by using anhydrous phenol. The following Table I sets forth the characteristics of six solvent extraction products which may be used in accordance with this invention. These are phenol extracts and were obtained during ordinary extraction practices as just described. The phenol extracts numbered 1-4 and 4a were prepared by treatment of bright stock from a Van Crude oil. These five extracts have flash points of from about 510°-550° F. and fire points of 590° or above. Phenol extract 5 is from a so-called neutral lubricating oil fraction. This extract is characterized by its lower viscosity. The flash point is 395° F. and the fire point up to 485° F. Throughout the balance of the specification these six extracts will be referred to by their corresponding numbers in the left-hand column of Table I. These extracts are listed as merely illustrative and the invention is not to

be limited thereby. It is to be understood that any solvent extract from the refining of a lubricating oil fraction for the purpose of separating paraffinic from non-paraffinic hydrocarbons will apply and be useful in the present invention. The characteristics of the extracts will depend on the type of solvent used and the type of lubricating oil fraction treated. It may be that the aromatic content of the extract is the solubilizing agent, for extreme pressure agents. However, the invention is not to be limited to any theory of solubilization.

stable in a Mid-Continent solvent refined bright stock in the same proportions by weight as shown by composition 7. Composition 8 shows that a high concentration of solvent refined 500 neutral has an adverse effect on the stability. The Gulf Coast 160 Bright is not a solvent refined oil and is completely compatible with the S-P lard oil. Even lowering the weight percent composition to 9% and using a less viscous extreme pressure base failed to give perfect compatibility as shown by composition 9. Composition 10 shows that 5% by weight of phenol

10

TABLE I  
*Characteristics of phenol extracts*

| No. | Source                               | API Gravity | Vis. 100° F. | Vis. 130° F. | Vis. 210° F. | V. I. | Pour °F. | Percent C. R. | Percent Sulphur |
|-----|--------------------------------------|-------------|--------------|--------------|--------------|-------|----------|---------------|-----------------|
| 1   | Bright Stock fr. Van Zandt Crude.    | 11.1        | 25,319       | 4,750        | 282          | -40   | +55      | 7.2           | 2.66            |
| 2   | do                                   | 13.7        | 25,000       | 5,400        | 355          | +27   | +80      |               | 2.18            |
| 3   | do                                   | 12.6        | 36,410       | 4,310        | 310.1        | -1    | +80      | 4.70          | 2.27            |
| 4   | do                                   | 14.6        | 19,500       | 4,305        | 313          | +27   | +90      | 4.7           | 2.27            |
| 4a  | do                                   | 15.4        | 32,500       |              | 372          | +5    | +60      | 4.13          | 2.33            |
| 5   | 160/180 Neutral fr. Van Zandt Crude. | 12.5        | 2936         | 322          | 61.5         | -38   | +50      | 0.29          | 2.49            |

The solubilizing effect of solvent extracts of lubricating oils on extreme pressure agents in lubricating oils of the solvent refined and Pennsylvania bright stock variety is best demonstrated by actual storage stability tests of different lubricating oil compositions. For this purpose various gear oil compositions have been used to demonstrate first the storage stability and insolubility problem and secondly its solution. Gear oil compositions are used as merely illustrative and the invention is not to be limited thereby. Table II following shows that with solvent refined bright stock the S-P lard oil is unstable. This phenomenon is not ordinarily experienced with solvent refined neutral stocks except highly viscous neutrals or stocks which are not solvent refined except the Pennsylvania bright stocks.

25 extract 1 is insufficient to obtain storage stability and again demonstrates that for all practical purposes S-P lard oil is incompatible with a Mid-Continent solvent refined 150 bright stock.

30 80 grade gear oil compositions which meet MIL-L-2105 requirements must have a viscosity at 210° F. of from 55 to 65 SUS, a minimum viscosity index of 85 and a channel point of -30° F. maximum. 90 grade gear oils under MIL-L-2105 approval must have a viscosity at 210° F. of 80 to 90 and a minimum viscosity index of 85 and show a 0° F. maximum channel. 35 SAE requirements for 80 and 90 grade oils are not as severe as the military and conform to compositions intended for ordinary commercial use. Under SAE requirements a combination 80/90 grade gear oil should

TABLE II  
*Stability of S-P fatty oil E. P. agents in various hydrocarbon oil compositions*

| No. | Composition                                                                                                                                                                | Vis./<br>210° F. | Vis./<br>100° F. | V. I. | Pour<br>°F. | Storage Stability                     |            |          |
|-----|----------------------------------------------------------------------------------------------------------------------------------------------------------------------------|------------------|------------------|-------|-------------|---------------------------------------|------------|----------|
|     |                                                                                                                                                                            |                  |                  |       |             | R. T.                                 | 32° F.     | Days     |
| 6   | 18% S-P Lard Oil<br>82% Mid-Continent Solvent<br>Refined 200 Neutral.                                                                                                      | 64.7             |                  |       |             | OK                                    | OK         | 60       |
| 7   | 18% S-P Lard Oil<br>82% Mid-Continent Solvent<br>Refined Bright Stock.                                                                                                     | 169.6            |                  |       |             | Separation (noted drop in viscosity). | Separation | 60       |
| 8   | 12% S-P Lard Oil<br>2.5% Dibenzyl Disulfide<br>23% Gulf Coast 160 Bright<br>62.5% Mid-Continent Solvent<br>Refined 500 Neutral.                                            | 89.5             | 981              | 100   | +5          | OK                                    | Separation | 21       |
| 9   | 9% S-P Dioleate of Propylene<br>Glycol<br>1% Ortholeum 202<br>90% Mid-Continent Solvent<br>Refined Bright Stock.                                                           | 85.2             |                  |       |             | Trace<br>do                           | OK         | 30<br>60 |
| 10  | 9% S-P Lard Oil<br>1% Ortholeum 202<br>5% Phenol Extract #1<br>43% Mid-Continent Solvent<br>Refined 150 Bright Stock.<br>42% Mid-Continent Solvent<br>Refined 200 Neutral. | 87.7             | 900              | 105   | +20         | Heavy Separation<br>in 48 hrs.        | OK         | 60       |

A compatible gear oil composition will show no change in viscosity or separation of insolubles during storage at room temperature and 32° F. for 60 days. A drop in viscosity is an indication of a tendency to separation. A composition should pass both the room temperature test and the 32° F. test to be acceptable. Percentages shown are weight percent. Table II reveals that Mid-Continent solvent refined 200 neutral is compatible with sulfurized-phosphorized lard oil extreme pressure base (composition 6). However, the same extreme pressure base as in composition 6 proved to be un-

70 have a viscosity of between 800 to 1500 SUS at 100° F., an extrapolated viscosity at 0° F. of 100,000 maximum and a channel below -20° F. Military requirements for storage stability are described in test procedure CRC-L-22-445 and require no precipitation of sludge or separation during storage for 60 days at room temperature and 32° F.

75 Table III following shows certain combinations of 80 and 90 grade gear oil compositions using various solvent extracts described in Table I. Compositions 11 through 18 are 90 grade and compositions 19 and 20 are so-called

80/90 grade combination. Table III demonstrates that both SAE and military requirements for cold weather operation and storage stability may be met by the present compositions. By the addition of from 0.5 to 2.5 weight per cent of a pour depressant like Acryloid 150, a resinous or polymer-like ester of acrylic acid, such as methyl methacrylate polymers, in general those lubricating oil compositions containing up to 12% by weight of extreme pressure base may be made to meet the pour and channel requirements.

fluence the quantity and type of solvent extract useable to attain a balanced composition. The upper limit of the amount of solvent extract used in a given formulation is governed primarily by the V. I., pour and channel characteristics desired in the finished blend. Solvent extracts often have high pour points because of their wax content, consequently too high a concentration of extract may raise the pour and channel points above acceptable limits. Dewaxing the extract lowers the pour and allows larger amount to be used in blending. We have found

TABLE III

SAE 80 and 90 grade gear oil compositions using  
solvent extract

| No. | Composition (wt. percent)                                                                                                                                                                                                                                              | Vis./100° F. | Vis./210° F.                   | V. I. | Pour,<br>° F. | Channel                           | CRC-L-22-445 Storage<br>Stability |        |      |
|-----|------------------------------------------------------------------------------------------------------------------------------------------------------------------------------------------------------------------------------------------------------------------------|--------------|--------------------------------|-------|---------------|-----------------------------------|-----------------------------------|--------|------|
|     |                                                                                                                                                                                                                                                                        |              |                                |       |               |                                   | R. T.                             | 32° F. | Days |
| 11  | 9% S-P Lard Oil, Vis. 210/910<br>1% Ortholeum 202<br>15% Phenol Extract #2<br>25% High V. I. Bright<br>50% Raw Neutral (dewaxed)<br>9% S-P Lard Oil, Vis. 210/908<br>1% Dibenzyl Disulfide                                                                             | 1,246        | 93.7                           | 86    | 0             | -10° F.                           | OK                                | OK     | 60   |
| 12  | 11% Phenol Extract #3<br>22.5% High V. I. 150 Bright<br>56.5% Raw Neutral (dewaxed)<br>9% S-P Destearinized LPU Lard Oil<br>1% Ortholeum 202                                                                                                                           | 995          | 86.1                           | 91    | 0             | -10° F.                           | OK                                | OK     | 60   |
| 13  | 15% Phenol Extract #2<br>22% High V. I. 150 Bright<br>53% Raw Neutral (dewaxed)<br>12% S-P Lard Oil, Vis. 210/908<br>1% Dibenzyl Disulfide                                                                                                                             | 1,247        | 93.8                           | 86    | -10           | -20° F.                           | OK                                | OK     | 60   |
| 14  | 9% Phenol Extract #3<br>18.5% High V. I. 150 Bright<br>59.5% Raw Neutral (dewaxed)<br>12% S-P Lard Oil, Vis. 210/908<br>1% Ortholeum 202                                                                                                                               | 970.0        | 88.2                           | 98    | +15           | 0° F.                             |                                   |        |      |
| 15  | 9% Phenol Extract #3<br>18.5% High V. I. 150 Bright<br>59.5% Raw Neutral (dewaxed)<br>*12% S-P Lard Oil, Vis. 210/384<br>1% Dibenzyl Disulfide                                                                                                                         | 1,040.0      | 89.4                           | 94.0  | 10            | 0° F.                             |                                   |        |      |
| 16  | 14% Phenol Extract #4<br>14% High V. I. 150 Bright<br>59% Raw Neutral (dewaxed)<br>*Addition of 0.1% Acryloid 150 to above blend<br>12% S-P Lard Oil, Vis. 210/908<br>1% Dibenzyl Disulfide                                                                            | 949          | 81.9                           | 86    | 5             | OK at -5° F., Channel at -10° F.  | OK                                | OK     | 45   |
| 17  | 10% Phenol Extract #4<br>14% High V. I. 150 Bright<br>63% Raw Neutral (dewaxed)<br>18% S-P Lard Oil, Vis. 210/908<br>1% Ortholeum 202                                                                                                                                  | 967          | 85.1                           | 92.0  | +5            | OK at -5° F., Channel at -7° F.   | OK                                | OK     | 45   |
| 18  | 10% Phenol Extract #2<br>71% Raw Neutral (dewaxed)<br>12% S-P Lard Oil, Vis. 210/261<br>1% Dibenzyl Disulfide<br>39% High V. I. 150 Bright                                                                                                                             | 999          | 84.7                           | 88    | +10           | 0° F.                             | OK                                | OK     | 30   |
| 19  | 15.7% Phenol Extract #5<br>31.8% Mid-Continent 160/180<br>0.5% Acryloid 150<br>12% S-P Lard Oil, Vis. 210/371<br>1% Dibenzyl Disulfide<br>30% High V. I. 150 Bright<br>34.2% 170/100 Neutral<br>5.0% Phenol Extract #2<br>17.1% Phenol Extract #5<br>0.7% Acryloid 150 | 806          | 85.0 (Vis./0° F. =<br>85,000)  | 109   |               | -15° F.                           |                                   |        |      |
| 20  |                                                                                                                                                                                                                                                                        | 849          | 85.1 (Vis./0° F. =<br>100,000) | 104   |               | OK at -14° F., Channel at -18° F. |                                   |        |      |

Table III shows that the proper combination of ingredients to form a compatible composition is dependent on at least four factors: the viscosity of the extreme pressure additive, the characteristics of the solvent extract, the type of mineral lubricating oil, and the desired physical properties of the finished blend. Extreme pressure additives prepared in accordance with United States Patent 2,211,306 have relatively low viscosities, as 300 to 700 SUS/210° F. and are generally more compatible on blending than additives prepared in accordance with United States Patent 2,483,571, wherein the reaction is conducted with air bubbling therethrough and the product has a viscosity of 900 to 1200 SUS/210° F. The physical characteristics of the extract itself influence its ability to overcome storage instability and these characteristics may vary with the extraction process. The desired physical properties of the finished blend also in-

60 that acceptable formulations may be prepared using from 9% to 30% by weight of solvent extract, however these proportions are subject to the factors above mentioned. The optimum limits of extract content for a given formulation may be determined by empirical testing.

65 70 grade universal gear lubricants for military use are intended to function when the prevailing atmospheric temperature is above 0° F. Under these conditions and considering that load pressures up to 400,000 p. s. i. and sliding velocities of 0 to 18,000 feet per minute are experienced on the gear surfaces of the modern transmission and differential, it is the practice to severely test gear lubricants as to their high speed and high torque characteristics. The high speed axle test is designated CRC-L-19-645 and the high torque axle test as CRC-L-20-545. The high speed test can be passed by incorporating compounds like Ortholeum 202 and di-

benzyl disulfide in the composition. Ortholeum 202 is a sulfurized terpenic compound the preparation of which is described in United States Patent 2,443,823. Compositions prepared in accordance with this invention meet these high speed and high torque tests.

One of the final requirements of a gear lubricant is the CRC-L-20-545 for determining load-carrying, wear, stability and corrosion characteristics under conditions of high torque and low speed. For the purpose of demonstrating that gear oils compounded in accordance with this invention are comparable with presently acceptable compositions, the following Table IV presents both CRC-L-20-545 and oxidation stability tests on composition Number 14 from Table III and a commercial gear oil A having the following composition (percent weight):

12% S-P lard oil  
1% dibenzyl disulfide  
0.9% acryloid 150  
41% Gulf Coast 160 Bright  
45.1% Mid-Continent conventionally refined 200 Neutral

TABLE IV

High torque-low speed and oxidation performance tests on 90 grade gear oils

| Composition No.                    | A                                            | 14                                  |
|------------------------------------|----------------------------------------------|-------------------------------------|
| CRC-L-20-545:                      |                                              |                                     |
| Gear Condition—                    |                                              |                                     |
| Pinion.....                        | Light wear, light stain on pins and washers. | light wear, light stain on washers. |
| Ring.....                          | light wear.....                              | light wear on pins.                 |
| Rating.....                        | pass.....                                    | pass.                               |
| Gear Oil Oxidation Stability test— |                                              |                                     |
| Thrust washer.....                 | thin black deposit.....                      | light brown coating.                |
| Sump deposit.....                  | trace sludge, no deposit, trace varnish.     | none.                               |
| Vis. Change/210° F.....            | 4%.....                                      | 6%.....                             |
| Rating.....                        | very good.....                               | excellent.                          |

20

25

35

40

From the above table it is apparent that gear oil composition 14, containing 9% by weight of phenol extract 3, is comparable to the reference oil A, which is an accepted product. The gear oil oxidation stability test is conducted in a device designed to simulate conditions in a power transmission unit. The gear oil is subjected to agitation by a rotating gear impeller in the presence of air while heated to a temperature of from about 275° to 325° F. for a period of about 17 hours. A bronze thrust washer is maintained adjacent the gear impeller to catalyze oxidation and simulate the bronze bearing surfaces present in a transmission. A thermal regulator is used to regulate the gear oil temperature. The gear oil oxidation tests in Table IV were conducted for 17 hours at 300° F. The test gives a direct indication of the ability of the gear oil to withstand actual operating conditions in a power transmission unit.

A combination 80/90 gear lubricant prepared in accordance with this invention and having the following composition:

BLEND NO. 21

12% S-P lard oil (vis./210=525)  
1.0% dibenzyl disulfide  
30 17% high V. I. 150 Bright stock  
48.5% 170/100 neutral  
21% phenol extract #4a  
0.5% acryloid 150

has been qualified and accepted by the Review Board of Army Ordnance. The following Table V gives the results of physical and performance tests conducted using the above blended gear lubricant.

TABLE V  
Physical and performance characteristics of blend No. 21

| Test                                       | Results                                                                                                                                                                                                                                                            | Requirements        |                        |             |
|--------------------------------------------|--------------------------------------------------------------------------------------------------------------------------------------------------------------------------------------------------------------------------------------------------------------------|---------------------|------------------------|-------------|
|                                            |                                                                                                                                                                                                                                                                    | MIL-L-2105          | SAE 80                 | SAE 90      |
| Gravity.....                               | 23.8.....                                                                                                                                                                                                                                                          |                     |                        |             |
| Flash.....                                 | 430° F.....                                                                                                                                                                                                                                                        | 325° F. (Min.)..... |                        |             |
| Vis./0° F., SUS.....                       | 90,000 (Ext.).....                                                                                                                                                                                                                                                 | 100,000 (Max.)..... |                        | 800-1,500.  |
| Vis./100° F., SUS.....                     | 821.....                                                                                                                                                                                                                                                           |                     |                        |             |
| Vis./130° F., SUS.....                     | 361.....                                                                                                                                                                                                                                                           | 80-90.....          |                        |             |
| Vis./210° F., SUS.....                     | 84.5.....                                                                                                                                                                                                                                                          | 85 (Min.).....      |                        |             |
| V. I.....                                  | 106.....                                                                                                                                                                                                                                                           |                     |                        |             |
| Pour, ° F.....                             | +15.....                                                                                                                                                                                                                                                           |                     |                        |             |
| Channel, ° F.....                          | Below -10° F.....                                                                                                                                                                                                                                                  | 0° F. (Max.).....   | Below -20° F.....      | Below 0° F. |
| Percent Phosphorus.....                    | 0.031.....                                                                                                                                                                                                                                                         |                     |                        |             |
| Percent Chlorine.....                      | Nil.....                                                                                                                                                                                                                                                           |                     |                        |             |
| Percent Lead.....                          | Nil.....                                                                                                                                                                                                                                                           |                     |                        |             |
| Percent Sulfur (Total).....                | 1.76.....                                                                                                                                                                                                                                                          |                     |                        |             |
| Percent Sulfur (in Mineral oil).....       | 0.73.....                                                                                                                                                                                                                                                          |                     |                        |             |
| Rust (Steel Strip, 4 hrs./150° F.).....    | Pass.....                                                                                                                                                                                                                                                          | Pass.....           |                        |             |
| Copper Strip Activity (1 hr./250° F.)..... | Stained (pass).....                                                                                                                                                                                                                                                | do.....             |                        |             |
| SAE/1,000 R. P. M.....                     | 130.....                                                                                                                                                                                                                                                           |                     |                        |             |
| SAE/500 R. P. M. (after heating).....      | 270.....                                                                                                                                                                                                                                                           |                     |                        |             |
| Timken:                                    |                                                                                                                                                                                                                                                                    |                     |                        |             |
| Beam Load (lbs.).....                      | 59.....                                                                                                                                                                                                                                                            |                     |                        |             |
| Pressure (p. s. i.).....                   | 32,000.....                                                                                                                                                                                                                                                        |                     |                        |             |
| Foam Test Sequence (1), Room Temp.....     | 0 cc.....                                                                                                                                                                                                                                                          | 650 cc. (Max.)..... |                        |             |
| CRC-L-20-545 Gear Condition.....           | Pinion Gear: Dull burnish, Medium wear. Ring Gear: Dull burnish, Light wear. (No surface fatigue on either, average back lash: 0.0001 inch increase, trace and light staining of differential gears, no deposits, discoloration or corrosion of axle shafts.)..... |                     |                        |             |
| Rating.....                                | Pass.....                                                                                                                                                                                                                                                          | Pass.....           |                        |             |
| CRC-L-19-645 Gear Condition.....           | (Duplicate runs): Ring and Pinion Gears Drive side, no scoring. Ring and Pinion Gears Coast side, no scoring.....                                                                                                                                                  |                     | Pass in duplicate..... |             |
| Rating.....                                | Pass.....                                                                                                                                                                                                                                                          |                     |                        |             |
| CRC-L-12-445:                              |                                                                                                                                                                                                                                                                    |                     |                        |             |
| Sequence (1), Room Temp.....               | 0 cc.....                                                                                                                                                                                                                                                          | 650 cc./Max.....    |                        |             |
| Sequence (2) 200° F.....                   | 50 cc.....                                                                                                                                                                                                                                                         | 650 cc./Max.....    |                        |             |

In Table V the CRC-L-20-545 Dynamometer Test, a high torque-low speed test, was conducted, using a Dodge  $\frac{3}{4}$  9 $\frac{1}{2}$  inch Hypoid axle, with the oil temperature at 200°-250° F. for 30 hours with 32,311 pound-inch torque at 62 revolutions per minute. The CRC-L-19-645 Dynamometer Test was conducted using a new Chevrolet Hypoid third member assembly with a 9-37 ratio in a dynamometer installation to simulate a Chevrolet passenger vehicle.

Although the invention has been demonstrated by specific examples it is not to be limited thereby and numerous ramifications may be practiced without departing from the sphere of the invention. The invention applies broadly to the use of solvent extracts from any lubricating oil fraction to impart solubility to extreme pressure agents especially those containing sulfur and phosphorus which are or tend to be insoluble in solvent refined lubricating oil fractions. For this result the amount of solvent extract used will be that amount which brings about the desired compatibility of the composition without deleteriously affecting other properties.

The following Table VI gives the characteristics of the lubricating oil fractions used herein. It is to be understood that the invention is not to be limited to compositions using the lubricants listed in Table VI, these being merely illustrative of the type of oils that may be used. It is also emphasized that the invention is not limited to lubricating compositions, as, those wherein a major portion is a lubricating oil. For example the solvent extracts may be used to dissolve the additive itself for use in subsequent compounding in a mineral lubricating oil. Also the solvent extracts may be added to lubricating oil fractions to make them compatible with extreme pressure additives.

We have also found that neutral stocks having viscosities of around 500 SUS at 100° F. are incompatible with S-P fatty bodies. One such oil is a Mid-Continent solvent refined 500 neutral. The invention applies with equal force to attaining compatibility on blends containing these high viscosity neutral stocks, as to the problem presented by solvent refined lubricating oils, especially the bright stocks and Pennsylvania bright stocks.

5

10

15

20

25

30

35

40

30

35

40

35

40

35

40

30

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35

40

35